



US005133900A

**United States Patent** [19]**Gallacher et al.****Patent Number:** **5,133,900****Date of Patent:** \* Jul. 28, 1992[54] **THERMOOXIDATIVELY STABLE COMPOSITIONS**[75] Inventors: **Lawrence V. Gallacher**, Norwalk, Conn.; **Alfen J. Gustavsen**, Ballwin, Mo.; **Robert L. Kugel**, Norwalk, Conn.[73] Assignee: **King Industries, Inc.**, Norwalk, Conn.

[\*] Notice: The portion of the term of this patent subsequent to Jan. 23, 2007 has been disclaimed.

[21] Appl. No.: **341,515**[22] Filed: **Apr. 21, 1989****Related U.S. Application Data**

[63] Continuation-in-part of Ser. No. 26,077, Mar. 16, 1987, Pat. No. 4,895,674.

[51] Int. Cl.<sup>5</sup> **C10M 135/18; C10M 135/10**[52] U.S. Cl. **252/400.52; 252/400.53; 252/400.61; 252/404; 252/406; 106/14.28; 106/14.29; 106/14.31**[58] Field of Search **525/18; 524/423; 252/401, 405, 387, 289.52, 389.62, 14.28, 389.52, 14.36, 404, 406, 400.52, 400.53, 400.61; 106/14.23, 14.36, 14.28, 14.29, 14.31**[56] **References Cited****U.S. PATENT DOCUMENTS**

- 2,840,477 6/1958 Shock et al. .... 106/14  
 2,856,362 10/1958 Morway ..... 252/33.3 X  
 3,090,250 5/1963 Bergen et al. .... 252/33.3 X  
 3,265,855 11/1966 Dexter et al. .... 252/57  
 3,285,855 11/1966 Spivack et al. .... 252/48.6  
 3,623,983 11/1971 Patten et al. .... 252/33.4  
 3,625,894 12/1971 Koenig et al. .... 252/33.4  
 3,629,109 12/1971 Gergel ..... 252/33.2 X  
 3,671,430 6/1972 Corringer ..... 252/33.3 X  
 3,684,726 8/1972 Haak et al. .... 252/33.2  
 3,763,042 10/1973 Gannon et al. .... 252/21  
 3,772,197 11/1973 Milsom ..... 252/33.2  
 4,125,479 11/1978 Chesluk et al. .... 252/336  
 4,201,681 5/1980 Lipinski et al. .... 252/33.2  
 4,213,892 7/1980 Scott ..... 260/45.95 C

- 4,326,972 4/1982 Chamberlin, III ..... 252/33.3  
 4,354,007 10/1982 Scott ..... 525/370  
 4,419,251 12/1983 Shim ..... 252/33.3 X  
 4,419,252 12/1983 Shim ..... 252/33.3 X  
 4,592,851 6/1986 Stadtmailler et al. .... 252/32.7 E

**FOREIGN PATENT DOCUMENTS**

- 471259 2/1949 Belgium  
 0295108 12/1988 European Pat. Off. ....  
 50-034003 7/1973 Japan .....  
 53-075137 4/1978 Japan .....

**OTHER PUBLICATIONS**

- Nose et al., Chemical Abstracts, 79 (26):147965h, "Oil Rustproofing Compositions," 1973, p. 82.  
 Chemical Abstracts, vol. 85, No. 4, Aug. 23, 1976, p. 151 Abstract No. 49156z, Institute of the Petrochemical and Gas Industry.  
 Chemical Abstracts, vol. 88, No. 2, Sep. 1, 1978, p. 147 Abstract No. 9571m, G. V. Barabanova.

*Primary Examiner*—Deborah L. Kyle*Assistant Examiner*—Valerie Fee*Attorney, Agent, or Firm*—Hedman, Gibson & Costigan

[57]

**ABSTRACT**

A composition which is thermooxidatively stable is provided which comprises a normally thermooxidatively unstable organic compound and effective amount of a thermooxidative stabilizing composition comprising an oil soluble sulfonate of a metal selected from barium, calcium, magnesium, zinc or a mixture of any of the foregoing; an effective amount of a stabilizer comprising an alkali or alkaline earth metal or zinc soap of an alkyl or alkenyl succinic acid, a partial ester thereof or a mixture of the foregoing; an effective amount of at least one primary antioxidant; optionally an effective amount of a secondary antioxidant; and optionally a carrier for the thermooxidative stabilizing composition. A thermooxidative stabilizing composition and a method for stabilizing a normally unstable organic compound comprising the addition of an effective amount of the thermooxidative stabilizing composition are provided as well.

**20 Claims, 1 Drawing Sheet**



FIG. 1

**THERMOOXIDATIVELY STABLE  
COMPOSITIONS**

**CROSS-REFERENCE TO RELATED  
APPLICATIONS**

This application is a continuation-in-part of copending U.S. patent application Ser. No. 07/026,077 filed on Mar. 16, 1987, U.S. Pat. No. 4,895,674. This application is also related to concurrently filed, copending U.S. patent application Ser. No. 07/341,516.

**FIELD OF THE INVENTION**

This invention relates to thermooxidatively stable sulfonate containing compositions. More particularly, it is concerned with the thermooxidative stabilization of normally thermooxidatively unstable organic compounds including both natural and synthetic media.

**BACKGROUND OF THE INVENTION**

Alkali metal and alkaline earth metal salts of high molecular weight alkaryl and petroleum sulfonic acids have long been widely used as dispersants and rust or corrosion inhibitors in a number of applications such as in lubricating oils, greases and rust-preventative coatings.

It has been reported that alkali metal and alkaline earth metal sulfonates can be combined with carboxylic acids, esters or soaps to enhance corrosion and oxidation inhibiting properties, e.g., U.S. Pat. Nos. 3,090,750; 3,625,894; 3,684,726; 3,763,042; 4,201,681; and Japanese Patent Publication 48/12238.

Bergen et al., U.S. Pat. No. 3,090,750, disclose greases which reform spontaneously upon cooling comprising an oil-insoluble metal compound, a dispersing agent selected from oil-soluble sulfonic acid or derivatives thereof or oil-soluble carboxylic acids or derivatives thereof, a lubricating oil and an acid coupling agent. Thermooxidative stability is not shown to be enhanced and synergism with antioxidants is not suggested.

In U.S. Pat. No. 3,625,894, Koenig et al. describe lubricating compositions combined with an anticorrosive consisting of an alkaline earth metal petroleum sulfonate and/or an oil-soluble alkaline earth metal salt of a C<sub>10</sub>-C<sub>36</sub> fatty acid and/or an oil-soluble alkaline earth metal salt of an alkylsulfamido-carboxylic acid, and benzotriazol. Although the compositions disclosed in the '894 patent are said to provide protection against corrosion for lubricants and mineral oils that have to withstand extreme temperatures, e.g., turbine oils, up to 170° C., only a temperature of 100° C. for 100 hours is exemplified. Furthermore, the use of primary antioxidants to provide synergism is not suggested.

Haak et al., U.S. Pat. No. 3,684,726 teach the inclusion of synergistic mixtures of barium alkaryl sulfonates and a naphthalene salt of zinc, lead, lithium or magnesium to improve the anti-corrosion properties of lubricating greases comprised of a metal soap and mineral oil. There is no disclosure in this patent however, that the thermooxidative stability of such greases is enhanced.

Gannon et al., U.S. Pat. No. 3,763,042, describe clay-thickened greases containing synergistic proportions of zinc dialkylnaphthalene sulfonate, an ester of an aliphatic monohydric alcohol and an aliphatic C<sub>12</sub>-C<sub>24</sub> monocarboxylic acid, zinc naphthenate, and other additives including certain other oxidation inhibitors. How-

ever, there is no exemplification of the combination with any oxidation inhibitors.

In U.S. Pat. No. 4,201,681, Lipinski et al. disclose a metal-working lubricant composition comprising a mineral oil and an additive combination of barium lanolate soap and barium sulfonate, e.g., barium didodecyl benzene sulfonate. The compositions of Lipinski et al. are tested for a number of characteristics, e.g., corrosion, stain and drawing properties, stack test for stain and friction measurements, visual observation for galling and scoring; however no enhanced stability to thermooxidation was investigated or demonstrated.

In Japanese Patent Publication No. 48/12238, published Feb. 15, 1973, as abstracted in CA 79(26):147965h, there are disclosed rustproofing oil compositions obtained by combining zinc soap of wool fatty acid and barium sulfonate to mineral oil. Improved rustproofing properties and moisture- and weathering-resistances are reported but no reference is made to rustproofing compositions having enhanced thermooxidative stability.

Stadtmailler et al., U.S. Pat. No. 4,592,851, disclose the use of a combination of a basic zinc dialkyl dithiophosphate and 2,6 di-t-butyl phenol to stabilize paraffinic mineral oil lubricants.

Dexter et al., U.S. Pat. No. 3,265,855, disclose the use of esters of hindered hydroxybenzoic and hydroxyphenyl alkanoic acids as stabilizers for organic materials subject to oxidative deterioration, and Scott, U.S. Pat. Nos. 4,213,892 and 4,354,007, discloses antioxidants as stabilizers for polymers, but neither suggest to combine these stabilizers with sulfonates.

It has now been unexpectedly discovered that the thermooxidative stability of normally thermooxidatively unstable organic compounds is remarkably and dramatically improved by the incorporation of a thermooxidative stabilizing composition comprising an oil-soluble barium, calcium, magnesium or zinc sulfonate; an alkali or alkaline earth metal or zinc soap of an alkyl or alkenyl succinic acid, a partially esterified alkyl or alkenyl succinic acid or a mixture of any of the foregoing; a primary antioxidant; optionally, a secondary antioxidant; and optionally a carrier for the thermooxidative stabilizing composition. When incorporated into normally thermooxidatively unstable organic compounds, oxidative degradation as well as deterioration caused by thermal effects are inhibited by the synergistic effect of the thermooxidative stabilizer composition or package components to a greater degree than is recognized in compositions of the prior art including those stabilized by a primary antioxidant and/or secondary antioxidants alone or oil soluble metal sulfonates stabilized by alkali or alkaline earth metal or zinc soap of alkyl or alkenyl succinic acid, partially esterified alkyl or alkenyl succinic acid or mixtures thereof alone.

It is a further object of this invention to provide a method for stabilizing a normally thermooxidatively unstable organic compound by blending the unstable compound and an effective amount of the thermooxidative stabilizing composition above.

This invention also contemplates thermooxidation stabilizer packages comprising only the thermooxidative stabilizer composition from above for use in the stabilization of normally thermooxidatively unstable organic compounds.

## BRIEF DESCRIPTION OF THE DRAWINGS

FIG. 1 is a graphic illustration of the synergistic effect of NA-SUL® ZS-HT—King Industries—Norwalk, Conn. (zinc dinonylnaphthalene sulfonate and zinc soap of the half methyl ester of dodecenylnsuccinic acid components) and primary antioxidant component of a thermooxidative stabilizing composition measured as the change in acid value (mg KOH/g) over time of a polyalphaolefin mixture in comparison with an unstabilized polyalphaolefin mixture and polyalphaolefin mixtures blended with either NA-SUL® ZS-HT or primary antioxidant alone.

## SUMMARY OF THE INVENTION

According to the present invention, there are provided thermooxidatively stabilized compositions comprising (A) a normally thermooxidatively unstable organic compound; and an effective amount of (B) a thermooxidative stabilizing composition comprising (i) an oil-soluble sulfonate of a metal selected from barium, calcium, magnesium, zinc or a mixture of any of the foregoing; (ii) an effective amount of a stabilizer comprising an alkali or alkaline earth metal or zinc soap of an alkyl or alkenyl succinic acid, a partially esterified alkyl or alkenyl succinic acid, or a mixture of any of the foregoing; (iii) an effective amount of at least one primary antioxidant; optionally, (iv) an effective amount of a secondary antioxidant; and optionally, (v) a carrier for the thermooxidative stabilizing composition.

The invention also provides a method for stabilizing a normally thermooxidatively unstable organic compound comprising blending with the compound, an effective amount of the thermooxidative stabilizing composition (B) from above.

Also contemplated by the invention are thermooxidative stabilizer compositions or packages comprising only component (B) from above.

## DETAILED DESCRIPTION OF THE INVENTION

Normally thermooxidatively unstable organic compounds which are used in the present invention include naturally occurring and synthetic organic compounds. These include, but not limited to, petroleum products, 45 lubricating oils of the aliphatic ester type, e.g., dihexyl azelate, di-(2-ethylhexyl)azelate, di-(3,5,5-trimethylhexyl)glutarate, diisoamyl adipate, pentacrythritol tetracaproate, triamyl tricarballylate, dipropylene glycol dipelargonate, 1,5-pentanediol di-(2-ethylhexanoate), and the like; animal and vegetable derived oils, e.g., linseed oil, fat, tallow, lard, peanut oil, cod liver oil, castor oil, palm oil, corn oil, cotton seed oil and the like; hydrocarbon material such as gasoline, both natural and synthetic, diesel oil, mineral oil, fuel oil, naphthenic oil, 55 drying oil, cutting fluids, waxes, resins and the like; fatty acids such as soaps; trimethylolpropane tripelargonate, EPT rubber, chlorinated rubber, natural rubber and the like.

Other materials thermooxidatively stabilized according to the present invention include cross-linked and thermoplastic resins having linear, branched and/or ring hydrocarbon sequences in the backbone or the side chain, and optionally substituted with, for example, oxygen, nitrogen and/or phosphorous; thermosetting polymers and various synthetic organic polymeric substances such as vinyl resins formed from the polymerization of vinyl halides or from the copolymerization of

vinyl halides with unsaturated polymerizable compounds, e.g., vinyl esters, alpha,beta-unsaturated acids, alpha,beta-unsaturated esters, alpha,beta-unsaturated ketones, alpha,beta-unsaturated aldehydes and unsaturated hydrocarbons such as butadienes and styrene; 5 polyalphaolefins such as polyethylene, polypropylene, polybutylene, polyisoprene and the like, including copolymers of poly-alpha-olefins, polyurethanes such as are prepared from polyols and organic polyisocyanates; polyamides such as polyhexamethylene adipamide; polyesters such as polymethylene terephthalates and polybutylene terephthalates; polycarbonates; polyacetals; polystyrene; polyethyleneoxide; and copolymers such as those of high impact polystyrene containing 10 copolymers of butadiene and styrene and those formed by the copolymerization of acrylonitrile, butadiene and/or styrene.

The barium, calcium, magnesium or zinc metal sulfonates useful as component (B)(i) in the practice of this invention include a wide variety of compounds known to those skilled in the art. The alkaryl or polyalkaryl sulfonates may be prepared by following the teachings of U.S. Pat. Nos. 2,764,548, 3,957,859, and 4,201,681.

Aromatic organic substrates, such as aromatic petroleum fractions, as well as benzene and its analogs, e.g., 25 alkylbenzenes, toluene, the xylenes, polyalkylbenzenes, and higher alkyl mono- and di- and polysubstituted benzenes, such as nonyl and decyl and dodecyl, straight and branched chain-substituted benzenes and the corresponding naphthalenes, form sulfonates which are preferentially oil soluble (selectively extractable with organic hydrocarbon solvents, and the like), and sulfonates which are preferentially water soluble (and alcohol soluble, being selectively extractable with water 30 and alcohols, and the like).

As is the case in U.S. Pat. No. 2,764,548, it is preferred to use a dinonylnaphthalene, the nonyl radicals of which are highly branched, and to use as a reaction solvent, a water-immiscible material selected from 40 naphtha, hexane, heptane, octane, chlorinated hydrocarbons and the like. Procedures to make the starting materials are thoroughly described in the '548 patent.

Methods for forming aromatic mono- and disulfonic acids, e.g., dinonylnaphthalene mono- and polysulfonic acids are well described in the aforementioned U.S. Pat. No. 3,957,859. Typically, these alkyl or polyalkylaryl sulfonic acids will have molecular weights in the range of greater than 150-2,500 or greater, preferably 200 or greater, most preferably 325 or greater. Suitable sulfonates are those having an alkaryl group, e.g., alkylated benzene or alkylated naphthalene. Illustrative examples of such sulfonic acids are dioctyl benzene sulfonic acid, didodecyl benzene sulfonic acid, dinonylnaphthalene sulfonic acid, dilauryl benzene sulfonic acid, lauryl cetyl benzene sulfonic acid, polyolefin alkylated benzene sulfonic acids such as polybutylene alkylated benzene sulfonic acid and polypropylene alkylated benzene sulfonic acid. Especially preferred as aromatic sulfonates in the practice of this invention are dinonylnaphthalene sulfonates, nonylnaphthalene sulfonates, petroleum sulfonates, dodecylbenzene sulfonates, and the like.

The metal salt or sulfonate salt (B)(i) is a salt of barium, calcium, magnesium, zinc or a mixture of any of the foregoing. The metal sulfonates of component (B)(i) may be formed by conventional methods known to those skilled in the art. The metal salts of aromatic sulfonic acids may be prepared by reacting an inorganic metal donor compound, e.g., metal hydroxide, metal

oxide or metal carbonate with the alkyl or dialkyl or polyalkyl aromatic sulfonic acid. Thus, for example, the reaction of any of barium hydroxide, calcium oxide, magnesium oxide, zinc hydroxide, and the like with the corresponding alkaryl sulfonic acid will yield suitable metal sulfonates. Suitable as component (B)(i) are barium, calcium, magnesium or zinc sulfonates such as barium dinonylnaphthalene sulfonate; calcium dinonylnaphthalene sulfonate; magnesium dinonylnaphthalene sulfonate; zinc dinonylnaphthalene sulfonate; barium alkylbenzene sulfonate, particularly barium dodecenylnaphthalene sulfonate; calcium alkylbenzene sulfonate, particularly calcium dodecenylnaphthalene sulfonate; magnesium alkylbenzene sulfonate, particularly magnesium dodecenylnaphthalene sulfonate; zinc alkylbenzene sulfonate, particularly zinc dodecenylnaphthalene sulfonate; or a mixture of any of these. Especially preferred are barium dinonylnaphthalene sulfonate, calcium dinonylnaphthalene sulfonate, magnesium dinonylnaphthalene sulfonate, and zinc dinonylnaphthalene sulfonate which are available under the respective tradenames NA-SUL® BSN, NA-SUL® CA, NA-SUL® MG, and NA-SUL® ZS, King Industries.

Contemplated for use as component (B)(ii) are alkali or alkaline earth metal or zinc soaps of an alkyl or alkenyl succinic acid, a partially esterified alkyl or alkenyl succinic acid or a mixture of any of the foregoing. Preferably, the alkyl or alkenyl succinic acid or the partially esterified alkyl or alkenyl succinic acid will have from 6 to about 50 carbon atoms, and most preferably will have from about 10 to about 30 carbon atoms.

The compounds useful as component (B)(ii) can be obtained by any known method but are generally obtained by reacting an inorganic metal donor compound, e.g., barium, calcium, magnesium or zinc and the like, with the appropriate alkyl or alkenyl succinic acid or partially esterified alkyl or alkenyl succinic acid. Preferred as component (B)(ii) are the barium soap of an alkenyl succinic acid, the barium soap of the half methyl ester of dodecenylnsuccinic acid, the calcium soap of an alkenyl succinic acid, the calcium soap of the half methyl ester of dodecenylnsuccinic acid, the magnesium soap of an alkenyl succinic acid, the magnesium soap of the half methyl ester of dodecenylnsuccinic acid, the zinc soap of an alkenyl succinic acid, the zinc soap of the half methyl ester of dodecenylnsuccinic acid or a mixture of any of the foregoing. Especially preferred are the barium, calcium, magnesium or zinc soaps of the half methyl ester of dodecenylnsuccinic acid. One convenient method of preparation is to react the alkyl or alkenyl succinic acid or corresponding anhydride or partial ester with a metal donor, such as barium hydroxide monohydrate, calcium oxide, magnesium oxide or zinc hydroxide monohydrate in the presence of a metal sulfonate (B)(i) and a small amount of lubricating oil at ambient or slightly elevated temperature.

The formed soap is then dehydrated by heating, and the lubricating oil component is added with stirring.

The primary antioxidants (B)(iii) of the present invention can be at least one phenolic antioxidant, at least one aromatic amine antioxidant, or a combination of any of the foregoing. Monophenols, bisphenols, thiobisphenols and polyphenols are all suitable phenolic antioxidants. Preferably, the phenolic antioxidant will comprise a hindered phenolic antioxidant, esters thereof including those disclosed in Dexter et al., U.S. Pat. No. 3,285,855, or a combination of any of the foregoing. Examples of suitable primary antioxidants are methylene bis-4,4'-2,6-

di-t-butyl phenol, 4,4'-dioctyldiphenylamine, alkylated phenyl-alpha-naphthylamines, t-butyl phenol derivatives, alkylated diphenylamines, phenyl-alpha-naphthylamine, sulfur containing hindered bisphenols, or a mixture of any of the foregoing.

The synergistic effect of components (B)(i), (B)(ii), and (B)(iii) may optionally be enhanced by the additional synergism of an effective amount of a secondary antioxidant (B)(iv) with components (B)(i), (B)(ii) and (B)(iii). Such secondary antioxidant will typically comprise a thiocarbamate, a thioester, or a combination of any of the foregoing and preferably will comprise zinc diethylthiocarbamate



wherein R is C<sub>5</sub>H<sub>11</sub>; or zinc diethylthiocarbamate



wherein R is C<sub>4</sub>H<sub>9</sub>.

Typically, the optional carriers (B)(v) can comprise a synthetic hydrocarbon base fluid such as a polyalphaolefin or a mixture of polyalphaolefins, mineral oil, a wax, an ester, a halocarbon fluid, polyglycol, mixtures of any of the foregoing and the like. Preferred as carrier (B)(v) are crystalline wax, mineral spirits, or kerosene. Especially preferred as carrier (B)(v) are light mineral oil, polyalphaolefins or mixtures thereof.

The mineral oils useful in the composition of this invention as carriers will generally have a viscosity of at least about 30 SUS up to about 600 SUS at 100° F. (37.7° C.). More particularly the mineral oils will have a viscosity of from about 40 SUS to about 350 SUS at 100° F. (37.7° C.) and preferably from about 50 to about 150 SUS at 100° F. (37.7° C.). The term light mineral oil generally is accepted to mean an oil with a viscosity of less than about 150 SUS at 100° F.

The mineral oils can vary widely in refinement, and they can be derived from a variety of crudes including paraffinic, naphthenic, asphaltic or mixed base. The mineral oils can be treated by any of the conventional refining methods including hydrogen treating, acid treating, extraction, etc., and blends or mixtures of such mineral oils can also be used.

Preferably, component (A) will comprise from about 95 to about 99.95 percent by weight and component (B) will comprise from about 5 to about 0.05 percent; by weight of (A) and (B) combined.

Preferably, component (B)(i) will comprise from about 2 to about 25 percent by weight, component (B)(ii) will comprise from about 3 to about 15 percent by weight; component (B)(iii) will comprise from about 20 to about 90 percent by weight; component (B)(iv) will comprise from zero to about 40 percent by weight; and component (B)(v) will comprise from zero to about 30 percent; by weight of (B)(i), (B)(ii), (B)(iii), (B)(iv) and (B)(v) combined.

Thermooxidative stability includes protection against thermal degeneration and oxidative degeneration.

The composition of the present invention can be employed in a number of applications including but not limited use, as compressor oils, engine oils, gear oils, hydraulic fluids, rust preventives, slushing oils, synthetic lubricants and turbine oils. In short, these compositions can be employed in any application requiring thermooxidative stability. These compositions are particularly useful in high temperature applications, e.g., greater than 150° C., especially greater than 180° C., and even greater than 200° C. for prolonged periods of time. Many of these compositions also exhibit enhanced rust and corrosion inhibiting properties.

A method of stabilizing normally thermooxidatively unstable organic compounds is also provided which comprises blending by any conventional means known to one of ordinary skill in the art such as mixing, stirring, dispersing, and the like, with the normally thermooxidatively unstable organic compound, an effective amount of the thermooxidative stabilizing composition or package (B) from above.

#### DESCRIPTION OF THE PREFERRED EMBODIMENTS

The following examples illustrate the invention without limitation. All parts and percentages are given by weight unless otherwise indicated. Induction period is the period of protection afforded against oxidation and/or increase in acid value.

Thermooxidative stability is reflected by change in acid value (mg KOH/g), color, sludge formation, length of induction period, change in viscosity, infrared absorption or a combination of any of the foregoing.

ASTM Test Method D4636-86 (a combination of Federal Test Methods 5307.1 and 5308.6) and a modified version of the IP48 test are incorporated in many of the examples below.

ASTM Test Method D4636-86 is conducted as follows:

200 ml of test sample are weighed into a large glass tube (cell) having an outside diameter of 51 mm and a length of approximately 350 mm exclusive of a large ground glass joint designed to accept an adapter head. The head, approximately 100 mm in height, contains standard taper ground glass joints for a reflux condenser, a thermowell and an O ring compression fit joint for accepting an air delivery tube. The thermowell is made of 5 mm OD glass tubing, is approximately 425 mm long, and comes to within 35 mm of the bottom of the tube. The temperature of the sample is monitored using a type J thermocouple attached to a remote thermometer. The air delivery tube is made of 6 mm OD glass tubing, is approximately 535 mm in length and is inserted to within 5 mm of the bottom of the tube. A flange is placed approximately 15 mm from the bottom of the air tube and on this flange are stacked in order, from the bottom, washer shaped specimens of aluminum alloy, silver, silicon-iron bronze, steel grade 1010, steel M50, magnesium, and titanium 8 percent manganese. The washers are 6.35 mm insider diameter by 19.05 mm outside diameter by 0.81 mm thick and are polished with 400 grit silicon carbide paper before use. Glass spacers, 9 mm OD and 6 mm in length, are used to separate the washers. Dry air is passed through the sample at 10±1 liters/hour.

The sample cells are immersed in high temperature silicone fluid, thermostatically heated in a Sta-Warm

heating bath. Samples are removed through the thermowell joint in the head through a U shaped tube approximately 600 mm long, to reach to the bottom of the main sample tube.

The modified IP48 test is conducted as follows:

36 grams of test sample are weighed into a large glass tube having an outside diameter of 38 mm and a length of approximately 200 mm exclusive of a standard taper ground glass joint at the top. An adapter containing a gas inlet tube, 8 mm OD, reaching to the bottom is inserted into the large glass tube, and a reflux condenser is fitted to the top. Lengths of copper and iron catalyst, each approximately 460 mm long, are braided around the gas inlet tube to form a tight coil approximately 50 mm long. The catalyst coil is activated by rinsing with heptane, air drying and immersing for one minute in a 15 v/v % solution of concentrated hydrochloric acid in acetone. After rinsing with water and then acetone, the coil is air dried.

The tube is immersed in a heating bath for 15 minutes and zero grade air is passed through the sample at 15 liters/hour.

#### PROCEDURE A

A 2000 ml flask with a heating mantle, stirrer, condenser and thermometer is charged with 750.1 grams of 40.5 percent active zinc dinonylnaphthalene sulfonate in naphthenic oil, 161.2 grams of dodecenyldsuccinic anhydride, 50 grams of 4 cSt synthetic hydrocarbon base fluid (polyalphaolein mixture—Emery ® 3004 PAO—Quantum Chemical Corp.—Cincinnati, Ohio, 20.8 grams of zinc oxide, and 200 grams of methanol and is stirred. The stirred reaction mixture is heated to reflux temperature and is held for two hours. The stirred reaction mixture is then heated to 150° C. under vacuum to strip the methanol, and the reaction product is polish filtered. The reaction product (NA-SUL ® ZS-HT—King Industries) is found to contain 31.36 percent zinc sulfonate and 18.24 percent zinc soap of the half methyl ester of dodecenyldsuccinic acid.

#### PROCEDURE B

A 1000 ml flask with a heating mantle, stirrer, condenser, and thermometer is charged with 339.6 grams of a 39.1 percent solution of dinonylnaphthalene sulfonic acid in heptane and 6.11 grams of low density magnesium oxide. A Dean-Stark trap is placed between the flask and the reflux condenser, and the reactants are heated with stirring to reflux temperature. After 1½ hours, water is removed from the reaction mixture to a pot temperature of 101° C. via the trap. The reaction product is cooled, and 165.4 grams of light mineral oil (75 sec. solvent extracted naphthenic oil—Telura ® 415—Exxon Company, USA—Houston, Tex.) is added. The heptane is stripped to a pot temperature of 150° C. under vacuum (25 torr). The reaction product is cooled to 65° C., and 68.8 grams of dodecenyldsuccinic anhydride; 100 grams of methanol and 5.5 grams of low density magnesium oxide is added. The resultant mixture is then heated to reflux temperature and is stirred for 2 hours. The stirred reaction mixture is then heated to 150° C. under vacuum to distill the methanol, and the reaction product is filtered. The concentrate (NA-SUL ® MG-HT—King Industries) is found to contain 34.33 percent magnesium sulfonate and 20.35 percent magnesium soap of the half methyl ester of dodecenyldsuccinic acid.

## PROCEDURE C

A 72 liter flask is charged with 13,986 grams of 50.7 percent solution of calcium dinonylnaphthalene sulfonate in naphthenic oil, 3626 grams of isohexadecenylsuccinic anhydride and 4000 grams of methanol and is stirred for 30 minutes. 535.0 grams of calcium hydroxide is added, and the stirred reaction mixture is heated to reflux temperature. After 4½ hours at reflux temperature, methanol is stripped at 150° C. under vacuum. 2697 grams of light mineral oil (75 sec. solvent extracted naphthenic oil—Telura® 415—Exxon Company, USA) is added and the resultant product is filtered. The reaction product (NA-SUL® CA-HT—King Industries) is analyzed by hyamine titration and HCl titration and is found to contain 33.94 percent calcium sulfonate and 25.19 percent of the calcium soap of the half methyl ester of isohexadecenylsuccinic acid.

## PROCEDURE D

A 2000 ml flask is charged with 700 grams of a 50.5 percent solution of barium dinonylnaphthalene sulfonate in naphthenic oil, 147.4 grams of isohexadecenylsuccinic anhydride, 200 grams of methanol and 100 grams of light mineral oil (75 sec. solvent extracted naphthenic oil—Telura® 415—Exxon Company, USA) and is blended. 55.6 grams of barium hydroxide monohydrate is added, and the stirred mixture is heated and is stirred at reflux temperature for 2 hours. Methanol is stripped at 150° C. under vacuum. An additional 56 grams of light mineral oil (75 sec. solvent extracted naphthenic oil—Telura® 415) is added, and the material is filtered. The reaction product is analyzed by hyamine titration and HCl titration and is found to contain 33.44 percent barium sulfonate and 23.42 percent of barium salt of the half methyl ester of isohexadecenylsuccinic acid.

## PROCEDURE E

A 1000 ml flask with a heating mantle, stirrer, condenser, and thermometer is charged with 75 grams of a 60 percent solution of dodecenylsuccinic acid in naphthenic oil and 225 grams of a overbased barium dinonylnaphthalene sulfonate in light mineral oil with a total base number of 48 and a sulfonate content of 45.7 percent (NA-SUL® BSB—King Industries). The contents of the flask are heated to 100° C. and are held for 1 hour with stirring to react the excess base in the sulfonate with the acid to form a mixture of barium soap and unreacted acid. The reaction mixture is then heated to 150° C. and stripped under vacuum, yielding 287 grams of reaction product. The reaction product is analyzed by acid-base titration and hyamine titration and is found to contain 4.23 percent free carboxylic acid, 16.32 percent of barium soap of dodecenylsulfonic acid and 36.42 percent of barium sulfonate. The resultant product is a clear, viscous brown liquid with an acid value of 16.7 mg KOH/g.

## EXAMPLE 1

A blend is prepared by dissolving 2.17 grams of the product prepared by the method of Procedure A (0.67 gram of zinc dinonylnaphthalene sulfonate, 0.38 gram of the zinc soap of the half methyl ester of dodecenylsuccinic acid, 1.12 grams of 4 cs synthetic hydrocarbon base fluid (polyalphaolefin mixture—Emery® 3004 PAO—Quantum Chemical Corp., (NA-SUL® ZS-HT—King Industries)) and 0.56 gram of primary antioxidant (4,4'-diocyldiphenylamine—Vanlube® 81—R. T. Vanderbilt Co.—Norwalk, Conn.) in 217.2 grams of solvent refined heavy paraffinic distillate (petroleum—Sunpar® LW110—Sun Refining and Marketing Company). 200 ml of the blend are placed in a test cell which is then exposed to a temperature of 150° C. under ASTM D43636-86 conditions. The initial blend is a light tan mobile liquid with an acid value of 0.78 mg KOH/g and a kinematic viscosity at 40° C. of 22.04 cSt. The induction period lasts through 185 hours. After 185 hours of exposure, the acid value is 0.83 mg KOH/g, and the viscosity at 40° C. was 21.801 cSt.

oxidant (methylene bis-4,4'-2,6-di-t-butyl phenol—Ethanox® 702—Ethyl Corp.—Baton Rouge—La.) in 217.2 grams of solvent refined heavy paraffinic distillate (petroleum—Sunpar® LW110—Sun Refining and Marketing Company—Philadelphia, Pa.). 200 ml of the blend are placed in a test cell which is then exposed to a temperature of 150° C. under ASTM D43636-86 conditions. The initial blend is a light tan mobile liquid with an acid value of 0.78 mg KOH/g and a kinematic viscosity at 40° C. of 22.04 cSt. The induction period lasts through 185 hours. After 185 hours of exposure, the acid value is 0.83 mg KOH/g, and the viscosity at 40° C. was 21.801 cSt.

## COMPARATIVE EXAMPLE 1A\*

200 ml of solvent refined heavy paraffinic distillate (petroleum—Sunpar® LW110—Sun Refining and Marketing Company) is placed in a test cell which is then exposed to a temperature of 150° C. under ASTM D4636-86 conditions. The initial sample is a colorless mobile liquid with an initial acid value 0.16 mg KOH/g and a kinematic viscosity at 40° C. of 20.67 cSt. After 16 hours, the sample turns orange, has an acid value of 3.67 mg KOH/g and has a viscosity at 40° C. of 27.30 cSt.

## COMPARATIVE EXAMPLE 1B\*

A blend is prepared by mixing 200 ml of solvent refined heavy paraffinic distillate (petroleum—Sunpar—LW110—Sun Refining and Marketing Company) and 0.4169 gram of primary antioxidant (methylene bis-4,4'-2,6-di-t-butyl phenol—Ethanox® 702—Ethyl Corp.). 200 ml of the blend are placed in a test cell which is then exposed to a temperature of 150° C. under ASTM D4636-86 conditions. The initial blend is a nearly colorless mobile liquid with an acid value of 0.16 mg KOH/g and a kinematic viscosity at 40° C. of 20.7 cSt. The induction period is 83 hours. After 185 hours of exposure, the acid value is 23.39 mg KOH/g, and the viscosity at 40° C. is 119.77 cSt.

## EXAMPLE 2

A blend is prepared by dissolving 2.7 grams of the product of Procedure A (0.67 gram of zinc dinonylnaphthalene sulfonate, 0.38 gram of the zinc soap of the half methyl ester of dodecenylsuccinic acid, 1.12 grams of 4 cSt synthetic hydrocarbon base fluid (polyalphaolefin mixture—Emery® 3004 PAO—Quantum Chemical Corp., (NA-SUL® ZS-HT—King Industries)) and 0.56 gram of primary antioxidant (4,4'-diocyldiphenylamine—Vanlube® 81—R. T. Vanderbilt Co.—Norwalk, Conn.) in 217.2 grams of solvent refined heavy paraffinic distillate (petroleum—Sunpar® LW110—Sun Refining and Marketing Company). 200 ml of the blend are placed in a test cell which is then exposed to a temperature of 150° C. under ASTM D4636-86 conditions. The initial blend is a light tan mobile oil with an acid value of 0.76 mg KOH/g and a kinematic viscosity at 40° C. of 22.09 cSt. The induction period lasts through 185 hours. After 185 hours of exposure, the sample turns to a brown clear liquid with an acid value of 0.89 mg KOH/g and a viscosity at 40° C. of 22.26 cSt.

## EXAMPLE 3

65 A blend is prepared by dissolving 0.56 gram of the product prepared by the method of Procedure A (0.174 gram of zinc dinonylnaphthalene sulfonate, 0.098 gram of the zinc soap of the half methyl ester of dodecenyl-

succinic acid, 0.288 gram of 4 cSt synthetic hydrocarbon base fluid (polyalphaolefin mixture—Emery® 3004 PAO—Quantum Chemical Corp.), (NA-SUL® ZS-HT—King Industries)) and 0.55 gram of primary antioxidant (4,4'-diocetylphenylamine—Vanlube® 81—R. T. Vanderbilt Co.) in 218.9 grams of solvent refined heavy paraffinic distillate (petroleum—Sunpar® LW110—Sun Refining and Marketing Company). 200 ml of the blend are placed in a test cell which is then exposed to a temperature of 150° C. under 10 ASTM D4636-86 conditions.

The initial blend is a nearly colorless mobile liquid with an acid value of 0.32 mg KOH/g and a kinematic viscosity at 40° C. of 21.35 cSt. The induction period lasts through 88 hours. After 88 hours of exposure, the 15 sample turns to a brown mobile liquid with an acid value of 0.41 mg KOH/g and a viscosity at 40° C. of 22.49 cSt.

#### EXAMPLE 4

A blend is prepared by dissolving 2.21 grams of the product of Procedure B (1.12 grams of magnesium dinonylnaphthalene sulfonate, 0.442 gram of the magnesium soap of the half methyl ester of dodecenylysuccinic acid, 0.708 gram of light mineral oil (75 sec. solvent extracted naphthenic oil—Telura® 415—Exxon Company, USA) (NA-SUL® MG-HT—King Industries)) and 0.55 gram of primary antioxidant (4,4'-diocetylphenylamine—Vanlube® 81—R. T. Vanderbilt Co.) in 217.2 grams of solvent refined heavy paraffinic distillate (petroleum—Sunpar® LW110—Sun Refining and Marketing Company). 200 ml of the blend are placed in a test cell which is then exposed to a temperature of 150° C. under ASTM D4636-86 conditions. The initial blend is a tan mobile liquid with an acid value of 0.25 mg KOH/g and a kinematic viscosity at 40° C. of 20.75 cSt. The induction period lasts through 72 hours. After 72 hours of exposure, the sample turns to a brown mobile liquid with an acid value of 0.62 mg KOH/g and a viscosity at 40° C. of 21.13 cSt.

#### EXAMPLE 5

A blend is prepared by dissolving 2.2 grams of the product of Procedure C (0.76 gram of calcium dinonylnaphthalene sulfonate, 0.45 gram of the calcium soap of the half methyl ester of dodecenylysuccinic acid, 0.99 gram of light mineral oil (75 sec. solvent extracted naphthenic oil—Telura® 415—Exxon Company, USA), (NA-SUL® CA-HT—King Industries)) and 0.55 gram of primary antioxidant (4,4'-diocetylphenylamine—Vanlube® 81—R. T. Vanderbilt Co.) in 217.2 grams of solvent refined heavy paraffinic distillate (petroleum—Sunpar® LW110—Sun Refining and Marketing Company). 200 ml of the blend are placed in a test cell which is then exposed to a temperature of 150° C. under ASTM D4636-86 conditions. The initial blend has an acid value of 0.32 mg KOH/g and a kinematic viscosity at 40° C. of 20.66 cSt. The induction period lasts 16 hours. After 16 hours of exposure, the acid value is 3.86 mg KOH/g and the viscosity is 24.45 cSt.

#### COMPARATIVE EXAMPLE 5A\*

A blend is prepared by mixing 200 ml of solvent refined heavy paraffinic distillate (petroleum—Sunpar® LW110—Sun Refining and Marketing Company) and 0.3793 gram of primary antioxidant (4,4'-diocetylphenylamine—Vanlube® 81—R. T. Vander-

bilt Co.). 200 ml of the blend are placed in a test cell which is then exposed to a temperature of 150° C. under ASTM D4636-86 conditions. The initial blend is a nearly colorless mobile liquid with an acid value of 0.14 mg KOH/g and a kinematic viscosity at 40° C. of 20.83 cSt. The induction period is 8 hours. After 16 hours, the acid value is 2.97 mg KOH/g, and the viscosity at 40° C. is 25.92 cSt.

#### EXAMPLE 6

A stock solution of 0.86 gram of calcium dinonylnaphthalene sulfonate and 0.60 gram of the calcium soap of the monomethyl ester of hexadecenylsuccinic acid in 1.0604 grams of light mineral oil (75 sec. solvent extracted naphthenic—Telura® 415—Exxon Company, USA) (NA-SUL® CA-HT—King Industries), 0.6291 gram of primary antioxidant (a sulfur containing hindered bisphenol—Irganox® L115—Ciba Geigy Corp.—Hawthorne, N.Y.), and 246.9 grams of light mineral oil (75 sec. solvent extracted naphthenic oil—Telura® 415) is prepared yielding a blend of 1 percent NA-SUL® CA-HT and 0.25 percent primary antioxidant. Approximately 36 grams of the blend are placed in each of five identical test cells and are exposed to a temperature of 150° C. under modified IP48 test conditions. Tubes are removed from the test bath at 16, 21, 26, 31 and 36 hours, and the changes in acid value (mg KOH/g) are -0.02, 0.13, 1.20, 1.21 and 1.32 respectively. No sludge is found in the 16 hour or 21 hour samples, but sludge is seen in the 26 hour sample indicating an induction period that lasts over 21 hours.

#### COMPARATIVE EXAMPLE 6A\*

A blend of a primary antioxidant (a sulfur-containing hindered bisphenol—Irganox® 415—Ciba Geigy Corp.) dissolved in 249.1 grams of light mineral oil (75 sec. solvent extracted naphthenic oil—Telura® 415—Exxon Company, USA) is prepared. Approximately 36 grams of blend are placed in each of five identical test cells and exposed to a temperature of 150° C. under modified IP48 test conditions. Tubes are removed from the test bath at 16, 22.5, 27.5, 32 and 37.5 hours, and the changes in acid value (mg KOH/g) are 0.41, 1.12, 1.66, 1.89, and 2.13 respectively. The 16 hour sample contains a trace of sludge, but the 22.5 hour sample has a film of sludge on the walls of the tube.

#### COMPARATIVE EXAMPLE 6B\*

A blend of 0.2471 grams of primary antioxidant (0.1212 gram of a 2,6-di-t-butyl phenol derivative—Irganox® L130—Ciba Geigy Corp. and 0.1259 gram of an alkylated phenyl-alpha-naphthylamine—Irganox® L57—Ciba Geigy Corp.) dissolved in 99.75 grams of light mineral oil (75 sec. solvent extracted naphthenic oil—Telura® 415—Exxon Company, USA) is prepared. 35.16 grams of the blend are placed in a test cell which is then exposed to a temperature of 150° C. under modified IP48 test conditions. The initial blend is a clear amber mobile liquid with an acid value of 0.16 mg KOH/g. After 65 hours of exposure, the acid value is 3.5 mg KOH/g, and a quantity of black sludge approximately 1 mm thick covers an area of approximately 20 cm<sup>2</sup> at the bottom of the test cell.

#### EXAMPLE 7

A stock solution of 7.04 grams of a blend of 2.47 grams of barium dinonylnaphthalene sulfonate and 1.41 grams of the barium soap of the half methyl ester of

dodecenyldsuccinic acid in 3.16 grams of naphthenic oil (NA-SUL® BSN-HT—King Industries) dissolved in 700.0 grams of light mineral oil (75 sec. solvent extracted naphthenic oil—Telura® 415—Exxon Company, USA) is prepared. 0.2505 gram of primary antioxidant (0.1251 gram of a 2,6-di-t-butyl phenol derivative—Irganox® L130—Ciba Geigy Corp. and 0.1254 gram of an alkylated phenyl-alpha-naphthylamine—Irganox® L57—Ciba Geigy Corp.) is dissolved in 99.75 grams of the stock solution yielding a blend containing 1 percent NA-SUL® BSN-HT and 0.5 percent primary antioxidant. 35.01 grams of the blend are placed in a test cell which is then exposed to a temperature of 150° C. under modified IP48 test conditions. The initial blend is a clear amber mobile liquid with an acid value of 0.35 mg KOH/g. After 65 hours of exposure, the acid value is 2.39 mg KOH/g, and a small quantity of black sludge is present in the bottom of the test cell having a thickness of less than 1 mm and an area of less than 3 cm<sup>2</sup>.

#### EXAMPLE 8

A blend is prepared by dissolving 2.2 grams of the product of Procedure D (0.75 gram of barium dinonylnaphthalene sulfonate, 0.44 gram of the barium soap of the half methyl ester of dodecenyldsuccinic acid, 1.01 grams of light mineral oil (75 sec. solvent extracted naphthenic oil—Telura® 415—Exxon Company, USA) (NA-SUL® BSN-HT—King Industries)) and 0.55 gram of primary antioxidant (4,4'-diocetylidiphenylamine—Vanlube® 81—R. T. Vanderbilt Co.) in 217.2 grams of solvent refined heavy paraffinic distillate (petroleum—Sunpar® LW110—Sun Refining and Marketing Company). 200 ml of the blend are placed in a test cell which is then exposed to a temperature of 150° C. under ASTM D4636-86 conditions. The initial blend has an acid value of 0.34 mg KOH/g and a kinematic viscosity at 40° C. of 20.80 cSt. The induction period lasts 16 hours. After 16 hours of exposure, the acid value is 2.72 mg KOH/g and the viscosity at 40° C. is 23.40 cSt.

#### EXAMPLE 9

A blend is prepared by dissolving 2.2 grams of the product of Procedure E (a partially neutralized 36.42 percent barium sulfonate, 16.32 percent barium soap of dodecenyldsuccinic acid composition, (NA-SUL® BSB-DA—King Industries)) and 0.55 gram of primary antioxidant (4,4'-diocetylidiphenylamine—Vanlube® 81—R. T. Vanderbilt Co.) in 217.2 grams of solvent refined heavy paraffinic distillate (petroleum—Sunpar® LW110—Sun Refining and Marketing Company). 200 ml of the blend are placed in a test cell which is then exposed to a temperature of 150° C. under ASTM D4636-86 conditions. The initial blend has an acid value of 0.45 mg KOH/g and a kinematic viscosity at 40° C. of 20.71 cSt. The induction period lasts 16 hours. After 16 hours of exposure, the acid value is 3.12 mg KOH/g and the viscosity at 40° C. is 23.95 cSt.

Examples 1, 2, 3, 4, 6 and 7 demonstrate the synergistic effect of components (B)(i), (B)(ii) and (B)(iii) of the present invention on the thermooxidative stability of petroleum compounds and mineral oils. When compared with Comparative Examples 1A\*, 1B\*, 5A\*, 6A\* and 6B\*, it is clearly shown that the synergism of the components provides enhanced thermooxidative stability over compositions containing none of components (B)(i), (B)(ii) or (B)(iii) or only component (B)(iii).

Example 6 provides better results than Example 5. Example 6 is performed under different test conditions with a different normally unstable organic compound than is Example 5. Example 7 provides better results than Examples 8 and 9. Example 7 is performed under different test conditions with a different normally unstable organic compound than Examples 8 and 9 as well.

#### EXAMPLE 10

A blend of 1 percent by weight of the product prepared by Procedure A (31.36 percent zinc dinonylnaphthalene sulfonate, 18.24 percent zinc soap of the half methyl ester of dodecenyldsuccinic acid, 50.40 percent 4 cs synthetic hydrocarbon base fluid (polyalphaolefin mixture—Emery® 3004 PAO—Quantum Chemical Corp.) (NA-SUL® ZS-HT—King Industries)), 0.25 percent weight of primary antioxidant (alkylated phenyl-alpha-naphthylamine—Irganox® LO6—Ciba Geigy Corp.), and 98.75 percent by weight of 4 cSt synthetic hydrocarbon base fluid (polyalphaolefin mixture—Emery® 3004 PAO—Quantum Chemical Corp. is prepared. 200 ml of the blend are placed in a test cell which is then exposed to a temperature of 175° C. under ASTM D4636-86 conditions. The induction period lasts over 88 hours. After 87 hours of exposure, there is no increase in acid value is (0.00 mg KOH/g), and the viscosity at 40° C. decreases 0.1 percent. Intermediate and final changes in acid value are illustrated in graph form in FIG. 1.

#### COMPARATIVE EXAMPLE 10A\*

200 ml of 4 cSt synthetic hydrocarbon base fluid (polyalphaolefin mixture—Synfluid® PAO 3004—Emery) are placed in a test cell which is then exposed to a temperature of 175° C. under ASTM D4636-86 conditions. There was no induction period. After 87 hours of exposure, the actual increase in acid value is 7.68 mg KOH/g, and the viscosity at 40° C. increases 261.3 percent. Intermediate and final changes in acid value are illustrated in graph form in FIG. 1.

#### COMPARATIVE EXAMPLE 10B\*

A blend of 1 percent by weight of the product prepared by the method of Procedure A (31.36 percent zinc dinonylnaphthalene sulfonate, 18.24 percent zinc soap of the half methyl ester of dodecenyldsuccinic acid, 50.40 percent 4 cSt synthetic hydrocarbon base fluid (polyalphaolefin mixture—Emery® 3004 PAO—Quantum Chemical Corp.) (NA-SUL® ZS-HT—King Industries)), and 99 percent by weight of 4 cs synthetic hydrocarbon base fluid (polyalphaolefin mixture—Emery® 3004 PAO) is prepared. 200 ml of the blend are placed in a test cell which is then exposed to a temperature of 175° C. under ASTM D4636-86 conditions. There is no induction period. After 87 hours of exposure, the actual increase in acid value is 6.86 mg KOH/g, and the viscosity at 40° C increases 23.8 percent. Intermediate and final changes in acid value are illustrated in graph form in FIG. 1.

#### COMPARATIVE EXAMPLE 10C\*

A blend of 0.25 percent by weight primary antioxidant (alkylated phenyl-alpha-naphthylamine—Irganox® LO6—Ciba Geigy Corp.) and 99.75 percent by weight of 4 cSt synthetic hydrocarbon base fluid (polyalphaolefin mixture—Emery® 3004 PAO—Quantum Chemical Corp. is prepared. 200 ml of the blend are placed in a test cell which is then exposed to

a temperature of 175° C. under ASTM D4636-86 conditions. The induction period is 28 hours. After 88 hours of exposure, the actual increase in acid value is 5.47, and the viscosity at 40° C. increases 77.3 percent. Intermediate and final changes in acid value are illustrated in FIG. 1.

#### EXAMPLE 11

A blend of 1 percent by weight of the product prepared by the method of Procedure A (31.36 percent zinc dinonylnaphthalene sulfonate, 18.24 percent zinc soap of the half methyl ester of dodecenylysuccinic acid, 50.40 percent 4 cSt synthetic hydrocarbon base fluid (polyalphaolefin mixture—Emery® 3004 PAO—Quantum Chemical Corp. (NA-SUL® ZS-HT—King Industries)), 0.10 percent by weight of primary antioxidant (alkylated phenyl-alpha-naphthylamine—Irganox® LO6—Ciba Geigy Corp.), and 99.9 percent by weight of 4 cSt synthetic hydrocarbon base fluid (polyalphaolefin mixture—Emery® 3004 PAO) is prepared. 200 ml of the blend are placed in a test cell which is then exposed to a temperature of 175° C. under ASTM D4636-86 conditions. After 87 hours of exposure, the actual increase in acid value is 4.00 mg KOH/g. Intermediate and final changes in acid value are illustrated in graph form in FIG. 1.

#### EXAMPLE 12

A blend of 1 percent by weight of the product prepared by the method of Procedure A (31.36 percent zinc dinonylnaphthalene sulfonate, 18.24 percent zinc soap of the half methyl ester of dodecenylysuccinic acid, 50.40 percent 4 cSt synthetic hydrocarbon base fluid (polyalphaolefin mixture—Emery® 3004 PAO—Quantum Chemical Corp.) (NA-SUL® ZS-HT—King Industries)), 0.25 percent by weight of primary antioxidant (4,4'-dioctylphenylamine—Vanlube® 81—R. T. Vanderbilt Co.), and 98.75 percent by weight of 4 cSt synthetic hydrocarbon base fluid (polyalphaolefin mixture—Emery® 3004 PAO) is prepared. 200 ml of the blend are placed in a test cell which is then exposed to a temperature of 175° C. under ASTM D4636-86 conditions. The induction period lasts over 88 hours. After 88 hours, the actual increase in acid value is 0.01 mg KOH/g, and the viscosity at 40° C. increases 0.29 percent.

#### COMPARATIVE EXAMPLE 12A\*

A blend of 0.25 percent by weight of primary antioxidant (4,4'-dioctylphenylamine—Vanlube® 81—R. T. Vanderbilt Co.) and 99.75 percent by weight of 4 cSt synthetic hydrocarbon base fluid (polyalphaolefin mixture—Emery® 3004 PAO—Quantum Chemical Corp. is prepared. 200 ml of the blend are placed in a test cell which is then exposed to a temperature of 175° C. under ASTM D4636-86 conditions. There is no induction period. After 88 hours of exposure, the actual increase in acid value is 6.21, and the viscosity at 40° C. increases 121.1 percent.

#### EXAMPLE 13

A blend of 1 percent by weight of the product prepared by Procedure A (31.36 percent zinc dinonylnaphthalene sulfonate, 18.24 percent zinc soap of the half methyl ester of dodecenylysuccinic acid, 50.40 percent 4 cSt synthetic hydrocarbon base fluid (polyalphaolefin mixture—Emery® 3004 PAO—Quantum Chemical Corp. (NA-SUL® ZS-HT—King Industries)), 0.25 percent by weight of primary antioxidant (a t-butyl phenol derivative—Irganox® L130—Ciba Geigy Corp.) and 98.75 percent by weight of 4 cSt synthetic hydrocarbon base fluid (polyalphaolefin mixture—Emery® 3004 PAO) is prepared. 200 ml of the blend are placed in a test cell which is then exposed to a temperature of 175° C. under ASTM D4636-86 conditions. The induction period lasts over 76 hours. After 88 hours, the actual increase in acid value is 2.14 mg KOH/g, and the viscosity at 40° C. increases 8.4 percent.

percent by weight of primary antioxidant (a t-butyl phenol derivative—Irganox® L130—Ciba Geigy Corp.) and 98.75 percent by weight of 4 cSt synthetic hydrocarbon base fluid (polyalphaolefin mixture—Emery® 3004 PAO) is prepared. 200 ml of the blend are placed in a test cell which is then exposed to a temperature of 175° C. under ASTM D4636-86 conditions. The induction period lasts over 76 hours. After 88 hours, the actual increase in acid value is 2.14 mg KOH/g, and the viscosity at 40° C. increases 8.4 percent.

#### COMPARATIVE EXAMPLE 13A\*

A blend of 0.25 percent by weight of primary antioxidant (a t-butyl phenol derivative—Irganox® L130—Ciba Geigy Corp.) and 99.75 percent by weight of 4 cSt synthetic hydrocarbon base fluid (polyalphaolefin mixture—Synfluid® PAO 3004—Emery) is prepared. 200 ml of the blend are placed in a test cell which is then exposed to a temperature of 175° C. under ASTM D4636-86 conditions. The induction period lasts 26 hours. After 88 hours of exposure, the actual increase in acid value is 5.61 mg KOH/g, and the viscosity at 40° C. increases 95.9 percent.

#### EXAMPLE 14

A blend of 1 percent by weight of the product prepared by the method of Procedure A (31.36 percent zinc dinonylnaphthalene sulfonate, 18.24 percent zinc soap of the half methyl ester of dodecenylysuccinic acid, 50.40 percent 4 cSt synthetic hydrocarbon base fluid (polyalphaolefin mixture—Emery® 3004 PAO—Quantum Chemical Corp.) (NA-SUL® ZS-HT—King Industries)), 0.25 percent by weight of primary antioxidant (phenyl-alpha-naphthylamine—PANA—Aldrich Chemical Company—Milwaukee, Wis.—recrystallized) and 98.75 percent by weight of 4 cSt synthetic hydrocarbon base fluid (polyalphaolefin mixture—Emery® 3004 PAO) is prepared. 200 ml of the blend are placed in a test cell which is then exposed to a temperature of 175° C. under ASTM D4636-86 conditions. The induction period lasts over 88 hours. After 88 hours, the actual decrease in acid value is 0.05 mg KOH/g, and the viscosity at 40° C. increases 3.9 percent.

#### COMPARATIVE EXAMPLE 14A\*

A blend of 0.25 percent by weight of primary antioxidant (phenyl-alpha-naphthylamine—PANA—Aldrich Chemical Company—Milwaukee, Wis.—recrystallized) and 99.75 percent by weight of 4 cSt synthetic hydrocarbon base fluid (polyalphaolefin mixture—Emery® 3004 PAO—Quantum Chemical Corp. is prepared. 200 ml of the blend are placed in a test cell which is then exposed to a temperature of 175° C. under ASTM D4636-86 conditions. The induction period lasts 48 hours. After 88 hours of exposure, the actual increase in acid value is 4.27 mg KOH/g, and the viscosity at 40° C. increases 53.8 percent.

#### EXAMPLE 15

A blend of 1 percent by weight of the product prepared by the method of Procedure A (31.36 percent zinc dinonylnaphthalene sulfonate, 18.24 percent zinc soap of the half methyl ester of dodecenylysuccinic acid, 50.40 percent 4 cSt synthetic hydrocarbon base fluid (polyalphaolefin mixture—Emery® 3004 PAO—Quantum Chemical Corp. (NA-SUL® ZS-HT—King Industries)), 0.25 percent by weight of primary antioxi-

dant (1:1 wt. ratio blend of an alkylated diphenylamine—Irganox® L57—Ciba Geigy Corp. and and a sulfur containing hindered bisphenol—Irganox® L115—Ciba Geigy Corp.) and 98.75 percent by weight of 4 cSt synthetic hydrocarbon base fluid (polyalphaolefin mixture—Emery® 3004 PAO) is prepared. 200 ml of the blend are placed in a test cell which is then exposed to a temperature of 175° C. under ASTM D4636-86 conditions. The induction period lasts over 111 hours. After 166 hours of exposure, the actual increase in acid value is 4.81 mg KOH/g, and the viscosity at 40° C. increases 30.4 percent.

#### COMPARATIVE EXAMPLE 15A\*

A blend of 0.25 percent by weight of primary antioxidant (1:1 wt. ratio blend of an alkylated diphenylamine—Irganox® L57—Ciba Geigy Corp. and a sulfur containing hindered bisphenol—Irganox® L115—Ciba Geigy Corp.) and 99.75 percent by weight of 4 cSt synthetic hydrocarbon base fluid (polyalphaolefin mixture—Emery® 3004 PAO—Quantum Chemical Corp.) is prepared. 200 ml of the blend are placed in a test cell which is then exposed to a temperature of 175° C. under ASTM D4636-86 conditions. The induction period lasts 70 hours. After 166 hours of exposure, the actual increase in acid value is 8.36 mg KOH/g, and the viscosity at 40° C. increases 78.1 percent.

Examples 10, 12, 13, 14, and 15 demonstrate the use of different primary antioxidants in achieving the synergistic effects of the present invention and of the application of the thermooxidative stabilizing package of the present invention in synthetic hydrocarbon base fluids.

Example 10, when compared with Comparative Examples 10A\*, 10B\* and 10C\* clearly demonstrates that the synergistic effect of components (B)(i), (B)(ii) and (B)(iii) (Example 10) result in superior thermooxidative stability to that which would result from just a combining effect of components (B)(i), (B)(ii) and (B)(iii). Comparative Example 10B\* indicates that the combination of components (B)(i) and (B)(ii) alone results in an acid value only 0.82 mg KOH/g less than the unstable organic compound, provides no induction period and results in a significant increase in viscosity at 40° C. Comparative Example 10C\* indicates that component (B)(iii) alone results in an acid value only 2.21 mg KOH/g lower than the unstable organic compound, provides no induction period and results in significant increases in viscosity at 40° C. Example 10, however, results in no increase in acid value, an 88 hour induction period and a decrease in viscosity. The synergistic effect of components (B)(i), (B)(ii) and (B)(iii) (Example 10) is greater than the mere combined effects of Comparative Example 10B\* and 10C\*.

Example 11 when compared with Example 10 illustrates that full synergism does not tend to occur if components are present in less than recommended amounts.

#### EXAMPLE 16

A blend of 75 grams of polyethylene (AC<sub>6</sub>—Allied Signal Corp.—Morristown, N.J.) and 75 grams of a different polyethylene (AC<sub>8</sub>—Allied Signal Corp.) is prepared. Brookfield viscosity at 140° C. is determined to be 350-40 cps. 0.1503 gram of primary antioxidant (methylene bis-4,4'-2,6-di-t-butyl phenol—Ethanox® 702 Ethyl Corp.) and 0.1529 gram of the product prepared by the method of Procedure A (31.36 percent zinc dinonylnaphthalene sulfonate, 18.24 percent zinc soap of the half methyl ester of dodecenylic acid,

50.40 percent 4 cSt synthetic hydrocarbon base fluid (polyalphaolefin mixture—Emery® 3004 PAO—Quantum Chemical Corp.) (NA-SUL® ZS-HT—King Industries)) are added to the blend. The resultant blend is placed in a test cell which is then exposed to a temperature of 175° C. under ASTM D4636-86 conditions. The initial sample of the resultant blend has an infrared absorbance of 0.040 at 1723 cm<sup>-1</sup>. The induction period is greater than 24 hours. After 24 hours of exposure, the sample has an infrared absorbance of 0.066 at 1718 cm<sup>-1</sup>.

#### COMPARATIVE EXAMPLE 16A\*

A blend of 75 grams of polyethylene (AC<sub>6</sub>—Allied Signal Corp.) and 75 grams of a different polyethylene (AC<sub>8</sub>—Allied Signal Corp.) is prepared and is placed in a test cell which is then exposed to a temperature of 175° C. under ASTM D4636-86 conditions. The initial sample has an infrared absorbance of 0.039 at 1722 cm<sup>-1</sup>, characteristic of the carbonyl group of carboxylic acids. The induction period is less than 16 hours. After 16 hours of exposure, the sample has an infrared absorption of 0.382 at 1722 cm<sup>-1</sup> indicating an increased carboxylic acid level.

#### COMPARATIVE EXAMPLE 16B\*

A blend of 75 grams of polyethylene (AC<sub>6</sub>—Allied Signal Corp.), 75 grams of a different polyethylene (AC<sub>8</sub>—Allied Signal Corp.) and 0.0912 gram of primary antioxidant (methylene bis-4,4'-2,6-di-t-butyl phenol—Ethanox® 702—Ethyl Corp.) is prepared and is placed in a test cell which is then exposed to a temperature of 175° C. under ASTM D4636-86 conditions. The initial sample has an infrared absorbance of 0.039 at 1722 cm<sup>-1</sup>. The induction period is less than 16 hours. After 16 hours of exposure, the sample has an infrared absorption of 0.190 at 1720 cm<sup>-1</sup>.

Example 16 and Comparative Examples 16A\* and 16B\* demonstrate the synergistic properties of component (B)(i), (B)(ii) and (B)(iii) when incorporated into thermoplastic polymers.

#### EXAMPLE 17

A blend of 0.2 percent by weight of the product prepared by the method of Procedure A (31.36 percent zinc dinonylnaphthalene sulfonate, 18.24 percent zinc soap of the half methyl ester of dodecenylic acid, 50.40 percent 4 cSt synthetic hydrocarbon base fluid (polyalphaolefin mixture—Emery® 3004 PAO—Quantum Chemical Corp.) (NA-SUL® ZS-HT—King Industries)), 0.15 percent by weight of primary antioxidant (4,4'-diethylphenylamine—Vanlube® 81—R. T. Vanderbilt Co.), 0.10 percent by weight of secondary antioxidant (zinc diamyldithiocarbamate, 50 percent active in oil—Vanlube® AZ—R. T. Vanderbilt Co.) and 99.65 percent by weight of 4 cSt synthetic hydrocarbon base fluid (polyalphaolefin mixture—Emery® 3004 PAO) is prepared. 200 ml of the blend are placed in a test cell which is then exposed to a temperature of 175° C. under ASTM D4636-86 conditions. The initial blend is a colorless mobile liquid with an acid value of 0.33 mg KOH/g and a kinematic viscosity at 40° C. of 16.94 cSt. The induction period lasts over 88 hours. After 88 hours of exposure, the acid value is 0.36 mg KOH/g, and the viscosity at 40° C. is 16.93 cSt.

#### COMPARATIVE EXAMPLE 17A\*

A blend of 1 percent by weight of the product prepared by the method of Procedure A (31.36 percent

zinc dinonylnaphthalene sulfonate, 18.24 percent zinc soap of the half methyl ester of dodecenyldsuccinic acid, 50.40 percent 4 cSt synthetic hydrocarbon base fluid (polyalphaolefin mixture—Emery ® 3004 PAO—Quantum Chemical Corp.) (NA-SUL ® ZS-HT—King Industries), 0.25 percent secondary antioxidant (zinc diamyldithiocarbamate, 50 percent active in oil—Vanlube ® AZ—R. T. Vanderbilt Co.) and 98.75 percent by weight of 4 cSt synthetic hydrocarbon base fluid (polyalphaolefin mixture—Emery ® 3004 PAO) is prepared. 200 ml of the blend are placed in a test cell which is then exposed to a temperature of 175° C. under ASTM D4636-86 conditions. The initial blend is a light tan mobile liquid with an acid value of 0.82 mg KOH/g and a kinematic viscosity at 40° C. of 16.96 cSt. The induction period lasts 5 hours. After 5 hours of exposure, the acid value is 6.47 mg KOH/g, and the viscosity at 40° C. is 20.67 cSt.

#### EXAMPLE 18

A blend of 0.05 percent by weight of the product prepared by the method of Procedure A (31.36 percent zinc dinonylnaphthalene sulfonate, 18.24 percent zinc soap of the half methyl ester of dodecenyldsuccinic acid, 50.40 percent 4 cSt synthetic hydrocarbon base fluid (polyalphaolefin mixture—Emery ® 3004 PAO—Quantum Chemical Corp.) (NA-SUL ® ZS-HT—King Industries), 0.15 percent by weight of primary antioxidant (4,4'-diocetylphenylamine—Vanlube ® 81—R. T. Vanderbilt Co.), 0.10 percent by weight of secondary antioxidant (zinc diamyldithiocarbamate, 50 percent active in oil—Vanlube ® AZ—R. T. Vanderbilt Co.), and 99.70 percent by weight of 4 cSt synthetic hydrocarbon base fluid (polyalphaolefin mixture—Emery ® 3004 PAO) is prepared. 200 ml of the blend are placed in a test cell which is then exposed to a temperature of 175° C. under ASTM D4636-86 conditions. The initial blend is a colorless mobile liquid with an acid value of 0.21 mg KOH/g and a kinematic viscosity at 40° C. of 16.94 cSt. The induction period lasts 72 hours. After 72 hours of exposure, the acid value is 3.18 mg KOH/g, and the viscosity at 40° C. is 19.29 cSt.

#### EXAMPLE 19

A blend of 1 percent by weight of the product prepared by the method of Procedure A (31.36 percent zinc dinonylnaphthalene sulfonate, 18.24 percent zinc soap of the half methyl ester of dodecenyldsuccinic acid, 50.40 percent 4 cSt synthetic hydrocarbon base fluid (polyalphaolefin mixture—Emery ® 3004 PAO—Quantum Chemical Corp.) (NA-SUL ® ZS-HT—King Industries), 0.25 percent by weight of primary antioxidant (alkylated phenyl-*alpha*-phanaphthylamine—Irganox ® LO6—Ciba Geigy), 0.25 percent by weight of secondary antioxidant (zinc diamyldithiocarbamate—Vanlube ® AZ—R. T. Vanderbilt Co.), and 98.5 percent by weight of 4 cSt synthetic hydrocarbon base fluid (polyalphaolefin mixture Emery ® 3004 PAO) is prepared. 200 ml of the blend is placed in a test cell which is then exposed to a temperature of 175° C. under ASTM D4636-86 conditions. The initial blend is a light tan mobile liquid with an acid value of 0.79 mg KOH/g and a kinematic viscosity at 40° C. of 17.23 cSt. The induction period lasts over 88 hours. After 88 hours of exposure, the acid value is 0.9 mg KOH/g, and the viscosity at 40° C. is 16.71 cSt.

Examples 17, 18 and 19 and Comparative Example 7A\* demonstrate the added synergistic effects of sec-

ondary antioxidants (B)(iv) when used in conjunction with components (B)(i), (B)(ii) and (B)(iii).

The above-mentioned patents and test methods are incorporated herein by reference.

Many variations will suggest themselves to those skilled in the art in light of the above detailed description. For example, instead of dinonylnaphthalene sulfonate, alkylbenzene sulfonate or petroleum sulfonate in component (B)(i), other sulfonates can be used, such as octyl, decyl, undecyl, dodecyl and the like. Likewise sulfonated diphenylalkanes can be used. Obviously, instead of diacids, the corresponding anhydrides and half esters can be used. Instead of mineral oil and polyalphaolefin as component (B)(v), other carriers, such as microcrystalline waxes, dioctyl adipate, silicone oils, and the like can be substituted. Other conventional additives can be added in conventional amounts, such as extreme pressure additives, dispersants and the like. All such obvious variations are within full intended scope of the appended claims.

We claim:

1. A composition comprising:

(A) an organic compound which is thermooxidatively unstable at temperatures greater than 150° C.; and

(B) a thermooxidative stabilizing composition to thermooxidatively stabilize said organic compound at temperatures greater than 150° C. comprising

(i) an oil soluble sulfonate of a metal selected from barium, calcium, magnesium, zinc or a mixture of any of the foregoing;

(ii) a stabilizer comprising an alkali or alkaline earth metal or zinc soap of an alkyl or alkenyl succinic acid, a partially esterified alkyl or alkenyl succinic acid or a mixture of any of the foregoing;

(iii) at least one primary antioxidant comprising a phenolic antioxidant, an aromatic amine antioxidant or a combination of the foregoing;

(iv) optionally a secondary antioxidant comprising a thiocarbamate, a thioester or a combination of the foregoing; and

(v) optionally a carrier, which may be the same as or different than said organic compound, for said thermooxidative stabilizing composition.

2. A composition as defined in claim 1 wherein component (A) is selected from the group consisting of a wax; an ester; a hydrocarbon fluid; a halocarbon fluid; a polyalphaolefin; a polyglycol; a mineral oil; a thermoplastic polymer; a thermosetting polymer; a copolymer of an olefin and a non-olefin; or a mixture of any of the foregoing.

3. A composition as defined in claim 1 wherein component (B)(i) comprises an oil soluble barium, calcium, magnesium, or zinc salt of an alkylarylsulfonic or petroleum sulfonic acid having a molecular weight above about 325.

4. A composition as defined in claim 3 wherein component (B)(i) comprises a barium, calcium, magnesium or zinc salt of a dialkylarylsulfonic acid.

5. A composition as defined in claim 4 wherein component (B)(i) comprises a barium, calcium, magnesium, or zinc salt of dinonylnaphthalene sulfonic acid.

6. A composition as defined in claim 1 wherein component (B)(i) is selected from the group consisting of barium dinonylnaphthalene sulfonate, calcium dinonylnaphthalene sulfonate, magnesium dinonylnaphthalene sulfonate, zinc dinonylnaphthalene sulfonate, barium alkylbenzene sulfonate, calcium alkylbenzene sulfonate,

magnesium alkylbenzene sulfonate, zinc alkylbenzene sulfonate, or a mixture of any of the foregoing.

7. A composition as defined in claim 1 wherein component (B)(ii) is selected from the group consisting of an alkali or alkaline earth metal or zinc soap of an alkyl or alkenyl succinic acid having from about 6 to about 50 carbon atoms, a partially esterified alkyl or alkenyl succinic acid having from 6 to about 50 carbon atoms, or a mixture of any of the foregoing.

8. A composition as defined in claim 1 wherein component (B)(ii) is selected from the group consisting of an alkali or alkaline earth metal or zinc soap of an alkyl or alkenyl succinic acid having from about 10 to about 30 carbon atoms, a partially esterified alkyl or alkenyl succinic acid having from about 10 to about 30 carbon atoms, or a mixture of any of the foregoing.

9. A composition as defined in claim 7 wherein component (B)(ii) comprises an alkaline earth metal soap of an alkenyl succinic acid.

10. A composition as defined in claim 7 wherein component (B)(ii) is selected from the group consisting of barium, calcium, magnesium or zinc soaps of an alkyl or alkenyl succinic acid, a partially esterified alkyl or alkenyl succinic acid or a mixture of any of the foregoing.

11. A composition as defined in claim 10 wherein component (B)(ii) is selected from the group consisting of a barium soap of an alkenyl succinic acid, a calcium soap of an alkenyl succinic acid, a magnesium soap of an alkenyl succinic acid, a zinc soap of alkenyl succinic acid, a barium soap of a partially esterified alkenyl succinic acid, a calcium soap of a partially esterified alkenyl succinic acid, a magnesium soap of a partially esterified alkenyl succinic acid, a zinc soap of a partially esterified alkenyl succinic acid, or a mixture of any of the foregoing.

12. A composition as defined in claim 10 wherein component (B)(ii) is selected from the group consisting of a barium soap of the half methyl ester of dodecenylnsuccinic acid, a calcium soap of the half methyl ester of dodecenylnsuccinic acid, a magnesium soap of the half methyl ester of dodecenylnsuccinic acid, a zinc soap of the half methyl ester of dodecenylnsuccinic acid, or a mixture of any of the foregoing.

13. A composition as defined in claim 1 wherein component (B)(ii) is selected from the group consisting of methylene bis-4,4'-2,6-di-t-butyl phenyl, 4,4'-dioctyldiphenylamine, alkylated phenyl-alpha-naphthylamine, t-butyl phenol derivatives, alkylated diphenylamines, phenyl-alpha-naphthylamine, sulfur containing hindered bisphenols, or a mixture of any of the foregoing.

14. A composition as defined in claim 1 wherein component (B)(iv) comprises a thiocarbamate.

15. A composition as defined in claim 1 wherein component (B)(iv) comprises zinc diamyldithiocarbamate.

16. A composition as defined in claim 1 wherein component (B)(v) is selected from the group consisting of waxes, esters, halocarbon fluids, polyalphaolefins, poly-

glycols, mineral oils, or mixtures of any of the foregoing.

17. A composition as defined in claim 1 wherein component (A) comprises from about 95 to about 99.95 percent by weight and component (B) comprises from about 5 to about 0.05 percent by weight of (A) and (B) combined.

18. A composition as defined in claim 1 wherein component (B)(i) comprises from about 2 to about 25 percent by weight; component (B)(ii) comprises from about 3 to about 15 percent by weight, component (B)(iii) comprises from about 20 to about 90 percent by weight; component (B)(iv) comprises from zero to about 40 percent by weight; and component (B)(v) comprises from zero to about thirty percent by weight of (B)(i), (B)(ii), (B)(iii), (B)(iv) and (B)(v) combined.

19. A method for stabilizing an organic compound which is thermooxidatively unstable at temperatures greater than 150° C. comprising blending with said compound, a thermooxidative stabilizing composition to thermooxidatively stabilize said organic compound at temperatures greater than 150° C. comprising:

- (i) an oil soluble sulfonate of a metal selected from barium, calcium, magnesium, zinc or a mixture of any of the foregoing;
- (ii) a stabilizer comprising an alkali or alkaline earth metal or zinc soap of an alkyl or alkenyl succinic acid, a partially esterified alkyl or alkenyl succinic acid or a mixture of any of the foregoing;
- (iii) at least one primary antioxidant comprising a phenolic antioxidant, an aromatic amine antioxidant or a combination of the foregoing;
- (iv) optionally a secondary antioxidant comprising a thiocarbamate, a thioester or a combination of the foregoing; and
- (v) optionally a carrier, which may be the same as or different than said organic compound, for said thermooxidative stabilizing composition.

20. A thermooxidative stabilizing composition to thermooxidatively stabilize an organic compound which is thermooxidatively unstable at temperatures greater than 150° C. comprising:

- (i) an oil soluble sulfonate of a metal selected from barium, calcium, magnesium, zinc or a mixture of any of the foregoing;
- (ii) a stabilizer comprising an alkali or alkaline earth metal or zinc soap of an alkyl or alkenyl succinic acid, a partially esterified alkyl or alkenyl succinic acid or a mixture of any of the foregoing;
- (iii) at least one primary antioxidant comprising a phenolic antioxidant, an aromatic amine antioxidant or a combination of the foregoing;
- (iv) optionally a secondary antioxidant comprising a thiocarbamate, a thioester or a combination of the foregoing; and
- (v) optionally a carrier, which may be the same as or different than said organic compound, for said thermooxidative stabilizing composition.

\* \* \* \* \*